

W. F. PRINCE.

PROCESS OF MELTING METAL CHIPS AND APPARATUS THEREFOR.

APPLICATION FILED NOV. 13, 1908.

Patented Oct. 5, 1909.

935,686.



Witnesses:

W. F. Kennedy  
Eleanor Vanderhof

Inventor:  
Walter F. Prince  
by his Atty:  
Philip George Prince Kennedy

# UNITED STATES PATENT OFFICE.

WALTER F. PRINCE, OF ELIZABETH, NEW JERSEY.

## PROCESS OF MELTING METAL CHIPS AND APPARATUS THEREFOR.

935,686.

Specification of Letters Patent.

Patented Oct. 5, 1909.

Application filed November 13, 1908. Serial No. 462,357.

To all whom it may concern:

Be it known that I, WALTER F. PRINCE, a citizen of the United States, residing at Elizabeth, county of Union, and State of New Jersey, have invented certain new and useful Improvements in Processes of Melting Metal Chips and Apparatus Therefor, fully described and represented in the following specification and the accompanying drawings, forming a part of the same.

This invention relates to a new method and apparatus for re-melting small pieces of cast iron or cast iron dust, and is especially intended for utilizing iron chips, such as borings, turnings, shavings and the like. Such iron chips have been handled in many different ways for re-melting, but all of these have proved unsatisfactory or uncommercial, on account of the results obtained or the cost.

In accordance with my invention, I fill the chips into sheet metal casings of such character that the heat required to melt the casing is considerably greater than that required to melt the cast iron chips, so that, in a furnace, the chips will be heated through the casings and brought into a pasty or semi-fluid state before the direct flame comes into contact with them by the melting of the casings. I preferably use wrought iron cylinders of convenient length, and melt the chips as part of a cupola charge, stacking the cylinders one on the other in the cupola charge. The transmission of heat through the casings brings the chips into condition to readily melt down with the rest of the cupola charge. The whole body of material in the furnace, therefore, settles down evenly, and, as the charging on top is continued, casings are added at the top and filled with chips. The chips may be used without any flux, or a flux may be mixed with the chips to reduce the melting point, and any ingredients required may be mixed with the chips to give the mixtures of melted iron desired. The casings thus form mixers in which the desired mixture of ingredients and their uniform distribution can be secured most conveniently and efficiently.

In the accompanying drawing forming a part of this specification, I have shown for the purpose of illustration a cupola charged with the chips added to a regular charge, in accordance with the preferred method of carrying out my invention, and the invention will now be explained in connection with

this drawing and the features forming the invention then specifically pointed out in the claims.

In the drawing, which is a vertical central section of a cupola broken away at the top, A is the cupola which is shown as of a common form and charged in the usual manner, except for the chip casings and their contents, *a* being the usual clay bed, *b* the successive bodies of coke, and *c* the successive bodies of iron to be melted. In the middle of the cupola are the casings 10 containing the cast iron chips 11, these casings being preferably wrought iron casings of from No. 18 to No. 24 gage, according to the heat to which the casings are subjected, and conveniently from twelve to twenty inches in diameter and from three to four feet long, although it will be understood that these dimensions may be varied. The casings may be open end cylinders, as shown, or may be closed at one end, so as to hold the chips independently of stacking the casings, or may be closed at both ends after filling.

In charging the cupola, the chips are preferably filled into the casings during charging, the bottom casing 10 being put into the cupola, preferably above the blast openings *d*, as shown, if the chips form only a part of a regular charge, so as to avoid the chips melting down before the rest of the charge, and filled with the chips, the cupola then charged to the top of this casing, and the second casing 10 added and filled with chips, the charging continued, and so on upward to the charging door. As the charge melts down with the casings and chips, the charging is continued, casings and chips being added at the top. Only one stack of chip casings is shown, but any number of stacks may be used in the cupola, according to the result desired. Any other method of charging may be used, however.

It is to be understood that the invention is not to be limited to the particular form of furnace shown but may be carried out in an apparatus of any suitable form, and that the casings of chips may be melted alone in a suitable cupola or other furnace, instead of in a regular furnace charge.

Although the invention is intended especially for treating iron chips, it may be applied to and includes the treatment of small pieces or dust of other metals, the casings being made of suitable metal to secure the results desired.

What I claim is:—

1. The method of melting iron chips and the like, which consists in packing the chips into casings having a sufficiently higher melting point than the chips so that the chips are melted by heat transmitted through the casings before the casings are melted, and melting the casings and chips in a suitable furnace.
- 10 2. The method of melting iron chips and the like, which consists in packing the chips into casings having a sufficiently higher melting point than the chips so that the chips are melted by heat transmitted through the casings before the casings are melted, and melting the casings and chips as part of the charge of a melting furnace.
- 15 3. The method of preparing iron chips and the like for melting, which consists in packing the chips into casings having a sufficiently higher melting point than the chips for the melting of the chips by heat transmitted through the casings before the casings are melted.
- 20 4. The method of preparing iron chips and the like for melting, which consists in charging a melting furnace and stacking one on the other in the charge successive chip-containing casings of metal having a sufficiently higher melting point than the chips for the melting of the chips by heat transmitted through the casings before the casings are melted.
- 25 5. The method of preparing iron chips and the like for melting, which consists in charging a melting furnace, stacking one on the other in the charge successive tubular casings of metal having a sufficiently higher melting point than the chips for the melting of the chips by heat transmitted through the casings and having open ends, and filling the successive casings with chips in charging the furnace.
- 30 6. A container for melting iron chips or the like, consisting of a casing of thin sheet metal having a melting point sufficiently higher than the chips to be melted, so that the chips may be melted by heat transmitted through the casings before the casings are melted.
- 35 7. A cupola furnace containing a charge of iron and fuel for melting and within the charge a series of casings mounted one upon the other and containing iron chips for remelting, said casings being of metal of a sufficiently higher melting point than the chips for the melting of the chips by heat transmitted through the casings.

In testimony whereof, I have hereunto set my hand, in the presence of two subscribing witnesses.

WALTER F. PRINCE.

Witnesses:

J. A. GRAVES,  
C. J. SAWYER.